

## UNITED STATES PATENT OFFICE

2,550,660

PROCESS FOR PRODUCING ADHERENT  
COATINGS ON STAINLESS STEEL TO  
FACILITATE DRAWING OPERATIONS

Paul Amundsen, Detroit, Mich., and John A. Henricks, Lakewood, Ohio, assignors, by mesne assignments, to Parker Rust Proof Company, Detroit, Mich., a corporation of Michigan

No Drawing. Application September 4, 1948,  
Serial No. 47,938

11 Claims. (Cl. 148—6.24)

1

The present invention relates to a novel process for producing adherent coatings on stainless steel to facilitate drawing operations. By the term "stainless steels" we mean steels which contain elements such as chromium with or without nickel, to prevent tarnish of the metal on exposure. Working of such steels in dies, particularly cold drawing in dies has been very difficult because of the nature of the surfaces of such stainless steels.

In cold drawing of carbon steels it has been found that drawing operations are facilitated by providing an adherent phosphate coating on the metal prior to the drawing operations. Attempts to produce a similar coating on stainless steel surfaces have not produced a coating having satisfactory properties of adherence, which at the same time will facilitate the cold drawing of the stainless steel material and thus facilitate the working thereof in drawing dies.

It is therefore, an important object of the present invention to provide a novel process for producing an adherent coating on stainless steel by chemical means, the process being readily adapted for use on an economically feasible basis in commercial scale operations.

It is a further object of the present invention to provide a novel process by which a chemically produced adherent coating is provided on stainless steel surfaces in a relatively short time, the produced coating being effective to improve the drawing properties of the stainless steel thus facilitating its cold drawing in manufacturing operations, increasing the life of the drawing dies and equipment and permitting the making of deeper draws in a single operation than has heretofore been possible in stainless steel drawing operations.

Other objects of the invention will appear in the following description and appended claims. Before explaining the present invention in detail it is to be understood that the invention is capable of other embodiments and of being practiced or carried out in various ways. It is also to be understood that the phraseology or terminology employed herein is for the purpose of description and not of limitation.

It has been observed heretofore that certain organic acids such as oxalic acid are, under certain conditions, very well suited for use in forming coatings on stainless steels in view of their known reactions therewith. It has been suggested in German Patent 731,045 that oxalic acid may be used with sulfides or hydrogen sulfide ( $H_2S$ ). While these solutions will form

2

coatings on the lower stainless steel alloys, the reaction requires a long time at high temperature. Some higher stainless steel alloys, especially the ones containing molybdenum, do not react to form any coating. As is known, hydrogen sulfide ( $H_2S$ ) is very poisonous and obnoxious and the difficulty in handling this material has made the process very impractical.

We have found that certain sulfur compounds which contain oxygen and which yield sulfur dioxide ( $SO_2$ ) and sulfur, can be used in the presence of oxalic acid and a soluble halide to form excellent coatings on stainless steel surfaces in a time interval of from about 2 to 10 minutes. Satisfactory compounds include thiosulfates, hydrosulfites, tetra-thionates and sulfites, together with alkali or ammonium halides such for example as sodium fluoride or bi-fluoride and/or sodium chloride.

The term "alkali" in the specification and appended claims is to include both the alkali metals and ammonium. The fluorides especially have proven to be effective and are preferred when high alloyed steels, containing molybdenum are to be coated.

Using such materials, a satisfactory coating is formed in 2 to 3 minutes at room temperature on 18-8 stainless steel. If the alloy contains molybdenum the temperature may be raised to 140°-150° F. in which event the time interval may be lengthened to 7 minutes.

The produced coatings are unlike coatings previously produced. On visual inspection they are dark gray in color. They are very adherent and form an ideal base for an additional conventional drawing compound or lubricant. For stainless steel tube drawing, a chlorinated wax emulsion has proven to be successful, whereas for stainless steel headlight rims, a simple soap solution such as sodium or potassium oleate in a dilute aqueous medium is satisfactory.

The concentration of the oxalic acid is not critical within the range of from approximately 2% to approximately 10%. The concentration of the other ingredients is not critical except that the sulfur compound should be kept below approximately 0.5%.

A typical working solution which has been found to give satisfactory coatings on stainless steel in several steel mills and automobile plants is made up as follows:

(Approx.) 5% oxalic acid, dihydrate  
(Approx.) 2% ammonium bi-fluoride  
(Approx.) 0.2%-0.5% sodium thiosulfate  
55 Water to make 100%

or

(Approx.) 5% oxalic acid  
 (Approx.) 2% sodium chloride  
 (Approx.) 1% sodium bi-fluoride  
 (Approx.) .2% sodium thiosulfate  
 Water to make 100%

Such a solution is heated to reactive temperatures, usually within the range of from approximately room temperature to approximately 190° F. and the properly cleaned stainless steel surfaces are immersed therein until a substantial coating is formed therein. This usually requires a time interval of from approximately 2 to approximately 10 minutes. The surfaces will be coated under these conditions and are then water rinsed and either dried or directly immersed in the drawing compound and subjected to the draw. In cleaning such surfaces they preferably are either alkali cleaned or pickled and water rinsed.

The solution as described above is tested for strength with N/10 sodium hydroxide, using a 5 ml. sample and methyl orange and phenolphthalein respectively. Such a solution tests free acid 23, total acid 34.5, ratio 1:1.6. This acid ratio slowly tends to increase to 1:2.0 and even higher. If it gets above 1:2.4 the coating action becomes sluggish, and this can be remedied by removing part of the sodium salts which crystallize out when the solution is cold, or by adding hydrochloric acid (HCl) or hydrofluoric acid (HF).

While we do not, at this time, fully understand all of the reactions which occur in such a process, it is our present belief that the soluble halide has an activator effect which overcomes the normal passivity of the stainless alloys and allows the coating reaction to be carried out much more rapidly and at much lower temperatures than in comparable processes in which the soluble halide is not used.

We do know however, that the use of the above activators for oxalic acid, causes the precipitation of an extremely smooth and adherent film of sulfide to be deposited on the surface, over which the normal coating of ferrous and other metal oxalates is formed. The sulfide containing film is in itself a lubricant and the more adsorptive normal type of oxalate which is formed, is heavier and seems to serve as an ideal base for the lubricant. It is possible to remove the top layer of the coating by polishing the surface, and the dark thin film of metallic sulfide is clearly visible.

We consider the function of the sulfur compound used to be that of a hydrogen depolarizer since hydrogen evolution is minimized, although this may be a matter of conjecture. Under certain conditions these compounds may be considered reducing agents, but we believe that their action here is more of an oxidizing nature.

As a class, we have found that the soluble halides are satisfactory activators and that of this group, the presently preferred soluble halides comprise the soluble alkali and ammonium salts of the fluorides and chlorides.

Having thus described the invention, what we desired to secure by Letters Patent of the United States is:

We claim:

1. In a process for treating the surfaces of stainless steel to facilitate cold drawing by producing an adherent coating thereon, the novel step of immersing the stainless steel in an

aqueous bath consisting essentially of oxalic acid, a sulfur compound containing oxygen which yields sulfur dioxide and sulfur under the conditions of the coating bath, and an activator consisting of a soluble alkali halide, for a time interval sufficient to form a substantial coating and at a reactive temperature within the range of from approximately room temperature to approximately 190° F.

2. In a process for treating the surfaces of stainless steel to produce an adherent coating thereon as claimed in claim 1 and further characterized in that the oxygen containing sulfur compound is selected from the group consisting of thiosulfates, hydrosulfites, tetra-thionates and sulfites.

3. In a process for treating the surfaces of stainless steel to produce an adherent coating thereon as claimed in claim 1 and further characterized in that the soluble halide is selected from the group consisting of the soluble alkali and ammonium salts of the chlorides or fluorides.

4. In a process for treating the surfaces of stainless steel to produce an adherent coating thereon as claimed in claim 3 and further characterized in that the soluble halide is an alkali fluoride.

5. In a process for treating the surfaces of stainless steel to produce an adherent coating thereon as claimed in claim 3 and further characterized in that the oxygen containing compound is selected from the group consisting of thiosulfates, hydrosulfites, tetra-thionates and sulfites.

6. A bath adapted to produce a coating on stainless steel surface and comprising an aqueous solution containing approximately 5% oxalic acid (dihydrate), approximately 2% ammonium bi-fluoride, 0.2% sodium thiosulfate and the balance water.

7. A bath adapted to produce a coating on a stainless steel surface and comprising an aqueous solution containing approximately 5% oxalic acid (dihydrate), 2% sodium chloride, 1% sodium bi-fluoride and 0.2% sodium thiosulfate and the balance water.

8. A bath adapted to produce a coating on stainless steel surfaces and comprising an aqueous solution containing approximately 5% oxalic acid (dihydrate), sodium thiosulfate in an amount ranging from approximately 0.2% to 0.5%, an activator selected from the group consisting of ammonium and sodium bifluoride in an amount of from approximately 1% to approximately 2%, and the balance water.

9. In a process for treating the surfaces of stainless steel to produce an adherent coating thereon the novel step of immersing the stainless steel in a bath containing approximately 5% oxalic acid (dihydrate), approximately 2% ammonium bi-fluoride, 0.2% sodium thiosulfate and the balance water for a time interval sufficient to form a substantial coating at a temperature within the range of from approximately room temperature to approximately 190° F.

10. In a process for treating the surfaces of stainless steel to produce an adherent coating thereon the novel step of immersing the stainless steel in a bath comprising approximately 5% oxalic acid (dihydrate), 2% sodium chloride, 1% sodium bi-fluoride and 0.2% sodium thiosulfate and the balance water, for a time sufficient to form a substantial coating at a temperature within the range of from approximately room temperature to approximately 190° F.

11. In a process for treating the surfaces of stainless steel to produce an adherent coating thereon the novel step of immersing the stainless steel in a bath containing approximately 5% oxalic acid (dihydrate), sodium thiosulfate in an amount ranging from approximately 0.2% to 0.5%, an activator selected from the group of ammonium and sodium bifluoride in an amount of from approximately 1% to 2% and the balance water, for a time interval sufficient to form a substantial coating at a temperature within the range of from approximately room temperature to approximately 190° F.

PAUL AMUNDSEN.

JOHN A. HENRICKS.

### REFERENCES CITED

The following references are of record in the file of this patent:

#### UNITED STATES PATENTS

| Number    | Name   | Date         |
|-----------|--------|--------------|
| 1,911,537 | Tanner | May 30, 1933 |

#### FOREIGN PATENTS

| Number  | Country | Date         |
|---------|---------|--------------|
| 554,280 | Germany | July 7, 1932 |
| 731,045 | Germany | Feb. 1, 1943 |